# EUROPEAN PATENT SPECIFICATION

(11) **EP 1 154 055 B1**
(45) Date of publication and mention of the grant of the patent: **09.07.2008**
(21) Application number: 00976251.9
(22) Date of filing: 15.11.2000
(51) Int. Cl.: D02G 3/02, D01F 6/62, D02G 1/02, D03D 15/00

(54) **POLYESTER YARN AND METHOD FOR PRODUCTION THEREOF**
POLYESTERGARN UND VERFAHREN ZUR SEINER HERSTELLUNG
FIL DE POLYESTER ET SON PROCEDE DE PRODUCTION

(30) Priority: 18.11.1999 JP 32794399
(43) Date of publication of application: 14.11.2001
(73) Proprietor: TORAY INDUSTRIES, INC., Tokyo 103-8666 (JP)
(72) Inventor: MOCHIZUKI, Katsuhiko, Toray Nakatogari Apt. 2-21, Sunto-gun, Shizuoka 411-0942 (JP); SUGANO, Koji, Toray Mishima-ryo E302, Mishima-shi, Shizuoka 411-0033 (JP); MAEDA, Yuhei, Toray Yoroizaka-shataku B82, Mishima-shi, Shizuoka 411-0033 (JP)
(74) Representative: Webster, Jeremy Mark
(86) International application number: PCT/JP2000/008040
(87) International publication number: WO 2001/036724

(56) References cited:
- WO-A1-99/27168
- JP-A- 11 100 747
- JP-A- 11 269 747
- JP-A- 11 302 932
- JP-A- 52 005 320

## Description

The present invention relates to polyester yarn comprising polytrimethylene terephthalate, and to a method for its production. More particularly, it relates to polyester yarn and to a method of producing polyester yarn which can be carried out stably at high speeds without package tightening and with little variation in properties in the fibre lengthwise direction and, furthermore, when the yarn is used to make a fabric, there is little sense of tightness because it stretches at a low modulus, and it has a soft handle.

Polytrimethylene terephthalate fibre is outstanding in its elastic recovery following elongation, possesses a low Young's modulus and soft bending characteristics and has good dyeing properties and, furthermore, chemically it has stable properties in the same way as polyethylene terephthalate. Hence, as may be seen for example from US-A-3584103 and US-A-3681188, it has long been the subject of research as a potential clothing material.

However, the starting material 1,3-propanediol is comparatively expensive, so polytrimethylene terephthalate has not been used as a synthetic fibre hitherto.

In recent years, as disclosed for example in US-A-5304691, a cheap method for the synthesis of 1,3-propanediol has been discovered, so the value of polytrimethylene terephthalate fibre has been re-examined.

According to investigations which we have carried out, if the two-stage method generally employed in the case of polyethylene terephthalate fibre is applied as it is to polytrimethylene terephthalate, directly after spinning there commences a change in internal structure and, as a result of a phenomenon referred to as package tightening, differences in properties arise due to differences in the extent of such changes in internal structure between the package inner and outer layers, and so fibre of stable quality is not obtained.

As a means for resolving this problem, there has been proposed a method using DSD in which the spinning process and drawing process are conducted continuously and, prior to winding-up, the internal structure is subjected to heat setting, as described in JP-A-52-008123. However, even by this method it has not been possible to suppress package tightening completely. EP-A-1033422 also proposes processes for producing PTT yarns.

The present invention has as its objective to provide a polyester yarn which shows no package tightening in the yarn production process so that a package of stable product quality is obtained and, furthermore, which has a low Young's modulus in the elastic recovery region, and is outstanding in its soft stretch properties and softness; together with a method for the production of this polyester yarn.

For the purposes of resolving the aforesaid problem, the present invention provides a polyester yarn which is a multifilament yarn substantially comprising polytrimethylene terephthalate and which has a strength from the stress-strain curve of at least 3 cN/dtex, a Young's modulus of no more than 25 cN/dtex, a minimum value of the differential Young's modulus at 3-10% extension of no more than 8 cN/dtex an elastic recovery following 10% elongation of least 90%, and a CV value of the continuous shrinkage in the yarn lengthwise direction of no more than 4%.

Furthermore, this polyester yarn can be obtained by a method of producing polyester yarn in which multifilament yarn obtained by the melt spinning of polymer substantially comprising polytrimethylene terephthalate having intrinsic viscosity [η] of at least 0.7 is hauled-off at a spinning rate of at least 2000 m/min and, without winding up, subjected to drawing and heat-treatment, after which it is continuously subjected to a relaxation heat treatment at a relaxation factor of 6 to 20% and wound-up as a package, wherein a textured roll of surface roughness 1.5S to 8S is used in the drawing and heat-treatment.

Moreover, according to another aspect, the present invention provides a woven fabric having such a polyester yarn as warp yarn and/or weft yarn in the form of a twisted yarn of twist coefficient 10,000 to 20,000.

Preferred embodiments of the invention will now be described in more detail with reference to the accompanying drawings and later with reference to Examples.

In the drawings:
Figure 1 is a schematic diagram showing an example of spin-drawing equipment for obtaining a polyester yarn embodying the present invention.
Figure 2 is a schematic diagram showing another example of spin-drawing equipment for obtaining polyester yarn embodying the present invention.
Figure 3 shows the stress-strain curve and the differential Young's modulus-strain curve for polyester yarn embodying the present invention (Example 1).
Figure 4 shows the stress-strain curve and the differential Young's modulus-strain curve for polyester yarn lying outside the present invention (Comparative Example 4).

### Explanation of the numerical codes

1: spinneret
2: cooling chimney
3: oiling guide
4: first heated roller
5: second heated roller
6: cooling roller
7: interlacing nozzle
8: winder

The polyester yarn of the present invention is multifilament yarn substantially comprising polytrimethylene terephthalate.

In the present invention, the polyester from which the polyester yarn is composed is polytrimethylene terephthalate (hereinafter abbreviated to PTT) where at least 90 mol% of the structural units are obtained from terephthalic acid as the chief acid component and 1,3-propanediol as the chief glycol component. However, there may be included copolymer components which can form other ester bonds, in a proportion which does not exceed 10 mol% and preferably does not exceed 6 mol%. Examples of copolymerizable compounds include dicarboxylic acids such as isophthalic acid, succinic acid, cyclohexanedicarboxylic acid, adipic acid, dimer acid, sebacic acid and 5-sodiumsulphoisophthalic acid, and diols such as ethylene glycol, diethylene glycol, dipropylene glycol, butanediol, neopentyl glycol, cyclohexanedimethanol, polyethylene glycol and polypropylene glycol.

Moreover, optionally, there may be added, for example, titanium dioxide as a delustrant, fine silica or alumina particles as a lubricant, hindered phenol derivatives as an antioxidant and colouring pigments.

It is important that the strength of the polyester yarn of the present invention be at least 3 cN/dtex. If the strength is less than 3 cN/dtex, as well as this leading to fuzzing and yarn breakages in subsequent processing stages such as weaving, the product obtained will also have reduced tear strength.

Furthermore, there is an inverse correlation between the extension at break and the frequency of occurrence of fuzzing at the time of weaving, and the higher the breaking extension while still satisfying the requirement in terms of practical strength, the more the occurrence of fuzzing can be suppressed. Hence, the residual extension is preferably at least 40% and more preferably at least 45%.

Again, it is important that the polyester yarn of the present invention has a Young's modulus of no more than 25 cN/dtex and that it has a minimum value of differential Young's modulus at 3-10% extension of no more than 8 cN/dtex. These properties are closely related to the elongation characteristics and the elastic recovery characteristics in a stretch fabric, and in order to attain the soft stretch property which is the objective of the present invention it is preferred that these properties have low values. That is to say, by satisfying all the above properties, when in the form of a fabric there is easy initial stretch (low Young's modulus) and, furthermore, within the extension range of 3-10%, which is the practical stretch recovery region, elongation is possible with no resistance (low differential Young's modulus). Hence, it is possible to produce a soft stretch fabric which is outstanding in its comfort when worn.

The Young's modulus has a linear relationship to the flexural stiffness of the fabric, and the lower the Young's modulus the more outstandingly soft is the fabric handle. Hence, the Young's modulus is preferably no more than 22 cN/dtex and more preferably no more than 20 cN/dtex.

In the same way, the minimum value of the differential Young's modulus at 3-10% extension is preferably no more than 5 cN/dtex.

The polyester yarn of the present invention has an elastic recovery of at least 90% following 10% elongation. If the elastic recovery is less than 90%, then there occurs the problem known as 'sagging' where, following elongation, there remains a portion which has undergone partial plastic deformation, so the woven material quality is reduced. The elastic recovery following 10% elongation is preferably at least 95% and more preferably at least 98%.

Now, the fact that yarn comprising PTT has outstanding elastic recovery is due to a considerable extent to its molecular structure. The reasons are thought to be because, in the crystal structure of PTT, the methylene chain of the alkylene glycol moiety has a gauche-gauche conformation, and interaction due to the stacking of benzene rings is low and the density low, so that flexibility is high, and hence the molecular chains readily stretch and recover by means of methylene chain rotation in the alkylene glycol moiety.

In experiments which we carried out, it was shown that the higher the degree of crystallinity the higher the elastic recovery. Consequently, the degree of crystallinity is preferably at least 30% and more preferably at least 35%. Here, the measurement of the degree of crystallinity was carried out based on the density in accordance with the density gradient column method of JIS L1013 (Chemical Fibre Filament Yarn Test Methods).

Furthermore, preferably, the boiling water shrinkage of the polyester yarn of the present invention is 3-15% and, moreover, the maximum value of the shrinkage stress is no more than 0.3 cN/dtex and the temperature at which the maximum value of shrinkage stress is shown is at least 120°C.

The boiling water shrinkage is one of the most important factors in terms of carrying out fabric design, and by making the boiling water shrinkage at least 3%, the setting properties are made favourable in subsequent processing stages, while by making it no more than 15% it is possible to obtain a fabric with a soft handle which is free of any sense of harshness. In the same way, if the heat shrink stress is too high, excess shrinkage will be introduced and the fabric handle will be harsh. Hence, in order to achieve a soft handle with no sense of harshness, the maximum value of the shrinkage stress is preferably no more than 0.3 cN/dtex and more preferably 0.15 to 0.25 cN/dtex. Again, the temperature at which the maximum value of shrinkage stress is shown is preferably at least 120°C and more preferably at least 130°C in order to facilitate subsequent processing such as setting and bulking-up.

In the case of the polyester yarn of the present invention, it is preferred that the CV% of the yarn lengthwise direction continuous shrinkage factor be no more than 4%. The CV% of the continuous shrinkage factor is an index of the uniformity of internal strain in the yarn lengthwise direction, and the smaller this value the higher the quality. In order to obtain fabric of high quality, the CV% is no more than 4%.

Again, it is preferred that the CF (coherence factor) value lies in the range 1-30, by subjecting the polyester yarn of the present invention to an interlacing treatment. Where the CF value is at least 1, it is possible to suppress single filament breakages at the time of yarn production and processing, and also at the time of weaving. Furthermore, where the CF value is no more than 30, when for example forming a combined yarn with different shrinkage as one component yarn, migration is facilitated, so this is preferred. It is further preferred that the CF value be 5 to 25.

The cross-sectional shape of the fibre from which the polyester yarn of the present invention is composed may be of circular cross-section, triangular cross-section, multilobal cross-section, flattened cross-section, X-shaped cross-section or other known profile section. Suitable selection may be made in accordance with the objectives.

Again, in order to enhance the softness when made into a woven fabric, the single filament fineness is preferably no more than 5 dtex and more preferably no more than 3 dtex.

In the case of the polyester yarn of the present invention, there is a strong correlation between the twist coefficient and the stretch property and, once the twist coefficient exceeds a fixed value, there is a tendency for the stretch property to increase rapidly. In practice, for a woven fabric employing yarn of twist coefficient about 5000, the percentage stretch is about 5%, but with a twist coefficient of 10,000 it is about 15% and with a twist coefficient of 14,000 it is about 30%. Hence, while the polyester yarn obtained in the present invention may be employed without twisting, it is more preferred that it be given a medium to hard twist with a twist coefficient of 10,000 to 20,000.

Now, the twist coefficient K is expressed by the relationship:- $twist coefficient K = T \times {D}^{0.5}$
where, T = number of twists per metre of yarn length and D = yarn fineness (decitex).

Here, T, the number of twists per metre of yarn length, is the value determined by untwisting the yarn with an electrically-powered twist detector under a 90 x 10⁻³ cN/dtex load, and dividing the number of 'untwists' when the yarn is completely untwisted by the yarn length following untwisting.

The form of the fabric of the present invention may be that of a woven material, knitted material, nonwoven material or cushion material, with suitable selection being made according to the objectives, and the fabric can be used, for example, in shirts, blouses, trousers, suits or blousons.

Next, an example of the method of producing the polyester yarn embodying the present invention is provided.

As a method for producing the PTT which is the starting material for a polyester yarn embodying the present invention, a method known as such may be employed. The intrinsic viscosity [η] of the PTT employed needs to be at least 0.7 in order to raise the spinnability at the time of yarn production and in order to obtain yarn of practical strength, but at least 0.8 is preferred.

Furthermore, in the production of a polyester yarn embodying the present invention, continuous polymerization and spinning may be employed whereby, following the polymerization, the polymer is directly subjected to spinning and drawing, or alternatively the polymer may first be converted into chip and dried, and then the spinning and drawing carried out.

The spinning temperature at the time of the melt spinning is preferably a temperature 10-60°C higher than the melting point of the PTT in order to stabilize the discharge from the spinneret, and more preferably the melt spinning is carried out at a temperature equal to the melting point plus 20 to 50°C. Again, in order to suppress oligomer deposition in the spinning and to enhance the spinning properties, there may be optionally provided 2-20 cm below the spinneret a heat shroud or suction device, or a means for generating an inert gas such as air, steam or nitrogen for preventing oxidative degradation of the polymer or spinneret contamination.

What is most important when producing a polyester yarn embodying the present invention is that the direct spin-draw method may be employed in which the drawing is immediately carried out following spinning, without temporarily winding-up.

In undrawn yarn comprising PTT, as stated above, a change in the internal structure begins immediately after spinning, with the phenomenon referred to as package tightening occurring, and this is a cause of differences in properties arising between the package inner and outer layers. When we carried out an investigation to suppress this package tightening, we found that an effective method comprises hauling-off the yarn at a spinning rate of at least 2,000 m/min and then, without temporarily winding up, immediately subjecting the yarn to drawing and heat treatment, after which it is continuously given a relaxation heat treatment by a relaxation factor of 5 to 20%. By using this method, the problem of package tightening is markedly improved, and it is possible to obtain yarn of high quality in which differences between the package interior and exterior layers are extremely small. Moreover, it has also been discovered that, by subjecting the yarn to a relaxation heat treatment at a high relaxation factor, there is obtained soft stretch yarn which is easily stretched and has a low Young's modulus in the elongation recovery region.

In order to reduce yarn unevenness and obtain uniform yarn which does not tend to show defects such as dyeing variations, it is important that the spinning rate be at least 2,000 m/min. By raising the spinning rate, the spinning tension is raised, and by making the yarn less susceptible to the effects of external disturbances the draw-down behaviour is made stable. Hence, the spinning rate is preferably at least 3,000 m/min. Furthermore, in order to secure stable spinnability, it is preferred that the spinning rate be no more than 6,000 m/min.

Again, it is preferred that the draw ratio be set such that the residual extension is at least 40%.

It is important that the relaxation factor at the time of the relaxation heat treatment following the drawing be made at least 6 to 20% in order to obtain the polyester yarn which is the objective of the present invention. By carrying out a relaxation heat treatment of at least 6% following drawing, it is possible to accelerate the relaxation of internal strain in the fibre, so the level of delayed relaxation of the residual strain is low and package tightening is suppressed. Furthermore, as explained above, by the relaxation heat treatment, elongation is facilitated in the practical extension range (up to 10% extension) and it is possible to confer outstanding characteristics in terms of soft stretch properties. It is further preferred that the relaxation factor be at least 8%. On the other hand, in order to achieve stability of yarn passage in the yarn production process, the relaxation factor is preferably no more than 20% and more preferably no more than 18%.

The relaxation heat treatment is now explained with reference to Figures 1 and 2.

Figure 1 is a schematic diagram of the method using a cooling roller in the relaxation heat treatment. Following discharge from spinneret **1,** cooling is carried out in chimney **2**, then convergence and oiling effected at oiling guide **3** and the yarn hauled-off and the temperature raised by first heated roller **4**, after which drawing and heat setting are performed between first heated roller **4** and second heated roller **5**. Furthermore, after passing through the drawing process, by employing the heat of second heated roller **5,** a relaxation heat treatment is carried out between the second heated roller **5** and cooling roller **6**, and winding-up performed by winder **8**. Now, in order to conduct the relaxation heat treatment still more efficiently, carrying out the relaxation treatment using a heat treatment means employing hot air or steam as a heating medium between the second heated roller **5** and cooling roller **6,** or carrying out the relaxation treatment in two stages by providing a third heated roller, are effective means for realizing the objective of the present invention.

Figure 2 is a schematic diagram of a method employing an interlacing nozzle in the relaxation heat treatment, and interlacing nozzle **7** has the role of a yarn cooling device and of a tension gradient controller. That is to say, by means of the interlacing treatment it is possible to lower the yarn tension prior to interlacing, so by utilizing the shrinkage stress produced by the heat of second heated roller 5 it is possible to perform a relaxation heat treatment between the second heated roller **5** and interlacing nozzle **7.** In such circumstances, the relaxation factor can be controlled by varying the actuating air pressure of the interlacing nozzle. Again, the relaxation treatment may also be carried out using a heat treatment means employing hot air or steam as a heating medium between the second heated roller **5** and interlacing nozzle **7,** or in two stages by providing a third heated roller.

In each case the relaxation factor is readily controlled and they are methods which are favourably employed in obtaining a polyester yarn embodying the present invention.

In the case of the heated roller (the second heated roller in the examples illustrated in Figure 1 and Figure 2) which serves both for the drawing and heat setting and for the relaxation heat treatment, there be used a textured roller of surface roughness 1.5S to 8S. The surface roughness is the section value of the maximum height (Rₘₐₓ) described in JIS B0601, and 1.5S to 8S in practice corresponds to the section values 1.6S, 3.2S, 6.3S. In terms of maximum height, this corresponds to more than 0.8 µm and up to 6.3 µm. By making the surface roughness at least 1.5S, the frictional coefficient between the yarn and roller is considerably reduced and there is a suitable degree of slip, so even at a high relaxation factor there is no winding of the yarn back on the heating roller, and stable yarn production is possible. As the surface roughness becomes higher, so yarn passage becomes more stable in the relaxation process but, if it exceeds 8S, the yarn surface is excessively abraded so a reduction in strength is brought about. The surface roughness of the heated roller is more preferably 3.2S to 6.3S (Rₘₐₓ: 1.7-6.3 µm). Now, the surface roughness is determined from measurement of the maximum height Rₘₐₓ using a Hommel Tester model T1000, made by the Hommel Co., based on JIS B0601.

In order to produce yarn stably without yarn breakages, the drawing temperature (the temperature of the first heated roller) is preferably 10-50°C higher than the glass transition temperature of the PTT, and more preferably the drawing is carried out at the glass transition temperature plus 20 to 40°C. The heat setting and relaxation heat treatment temperature (the temperature of the second heated roller) should be set within the range 90-180°C so as to achieve the desired percentage heat shrinkage but, in order to effect uniform relaxation of the residual stresses formed by the drawing, a temperature in the range 105-180°C is more preferred.

Furthermore, the spinning oil applied will contain, eg., lubricant, emulsifier and antistatic agent. Specifically, examples include mineral oils such as liquid paraffin, fatty acid esters such as octyl palmitate, lauryl oleate and isotridecyl stearate, dibasic acid diesters such as dioleyl adipate and dioctyl sebacate, esters of polyhydric alcohols such as trimethylolpropane trilaurate and coconut oil, aliphatic sulphur-containing esters such as lauryl thiodipropionate, nonionic surfactants such as polyoxyethylene oleyl ether, polyoxyethylene castor oil ether, polyoxyethylene nonyl phenyl ether and trimethylolpropane trilaurate, anionic surfactants such as alkyl sulphonate and alkyl phosphate type metal salts or amine salts, sodium dioctylsulphosuccinate and sodium alkanesulphonate and, for example, tetramethylene oxide/ethylene oxide copolymers and propylene oxide/ethylene oxide copolymers, and there is employed a formulation which enhances the passage through the yarn production, warping and fabric production stages, in particular passage through the reeds and heddles at the time of weaving. Where required, there may also be used, for example, rust preventives, antibacterial agents, antioxidants, penetrating agents, surface tension lowering agents, phase reversal viscosity lowering agents, wear preventing agents and other such modifiers.

From the point of view of passage through subsequent processing stages, the amount of oil applied is preferably 0.3 to 1.2 wt% in terms of the yarn.

### Examples

Below, embodiments of the present invention are explained in further detail by means of Examples. The various property values in the Examples were determined by the following methods.

### A. Intrinsic Viscosity [η]

Using an Ostwald viscometer, sample polymer was dissolved in o-chlorophenol (abbreviated below to OCP) and the relative viscosity ηᵣ determined at a number of points, after which the value at infinite dilution was obtained by extrapolation.

### B. Strength, Extension and Young's Modulus (initial resistance to stretching)

The sample was subjected to measurement using a Tensilon UCT-100 produced by the Orientec Co., under constant rate of elongation conditions as described in JIS L1013 (Chemical Fibre Filament Yarn Test Methods). The breaking extension was determined from the elongation at the point showing the maximum tenacity in the S-S curve.

Furthermore, the Young's modulus was measured under the conditions given for the initial resistance to stretching in 7.10 of JIS L1013 (Chemical Fibre Filament Yarn Test Methods).

### C. Differential Young's Modulus

This was determined by differentiation of stress with respect to extension at points on the S-S curve obtained in B.

### D. Elastic Recovery

Using a Tensilon UCT-100 produced by the Orientec Co. and with the clamp spacing at 20 cm, the sample was stretched to 10% of the clamp spacing at a rate of extension of 10 cm/min, then the load immediately removed at the same rate, and the elastic recovery determined from the hysteresis curve recorded. $elastic recovery ( % ) = ( β / α ) \times 100$
α: elongation when stretched 10%
β: recovered elongation up to the point when the stress equals the initial load

### E. Shrinkage Stress

Measurement was carried out at a rate of temperature rise of 2.4°C/sec using a thermal stress measurement device produced by Kanebo Engineering (Co.). The sample comprised a 2 x 10 cm loop and the initial tension = fineness (decitex) x 0.9 x (1/30) gf.

### F. CV% of Continuous Shrinkage Factor in Yarn Lengthwise Direction

Using an FTA500 made by the Toray Engineering Co., measurement was carried out with the set tension = fineness (decitex) x 0.9 x (1/60) gf, treatment temperature = 100°C (under steam), yarn velocity = 10 m/min and sample length = 10 m. The shrinkage was recorded on a chart and the CV% of the continuous shrinkage factor in the yarn lengthwise direction determined.

### G. CF Value

Measurement was carried out under the conditions shown for the Degree of Interlacing in 7.13 of JIS L1013 (Chemical Fibre Filament Yarn Test Methods). The CF value (coherence factor) was determined from the average value L (mm) of the length of the interlace using the following formula, based on 50 measurements. $CF value = 1000 / L$

### H. Degree of Crystallinity

The density was measured in accordance with the Density Gradient Column Method in 7.14.2 of JIS L1013 (Chemical Fibre Filament Yarn Test Methods) and the degree of crystallinity obtained by the following formula. ${X}_{c} [ % ] = \left\{{d}_{c}\times \left(d-{d}_{a}\right)\right\} / ( d \times \left({d}_{c}-{d}_{a}\right) } \times 100$
X_{c}: degree of crystallinity (%)
d: measured yarn density
d_{c}: density of completely crystalline region
dₐ: density of completely amorphous region

Here, d_{c} = 1.387 g/cm³, dₐ = 1.295 g/cm³

### Example 1

Using the spin-draw machine shown in Figure 1, homo-PTT of intrinsic viscosity [η] 0.96 was melted and spun from 24-hole spinneret **1** at a spinning temperature of 265°C and, after cooling in chimney **2** and then converging and oiling at oiling guide **3**, haul-off was performed at 3,000 m/min by means of first heated roller **4**, and having raised the temperature of the yarn by five laps at 70°C, drawing was carried out by means of second heated roller **5** at a drawing rate of 4800 m/min (draw ratio = 1.6). After heat-setting by five laps at 140°C, relaxation was performed by a relaxation factor of 10% between second heated roller **5** and cold roller 6, and then while performing an interlacing treatment at an actuating pressure of 0.2 MPa using interlacing device **7**, wind-up was performed at 4220 m/min with winder **8,** and **54** decitex, 24 filament, drawn yarn obtained. Now, for second heated roller **5** there was used a textured roll of surface hardness 3.2S (Rₘₐₓ: 3 µm).

The yarn production characteristics were good and there were no yarn breaks or filament wrap-around. Furthermore, the strength of the polyester yarn obtained was 3.6 cN/dtex, the Young's modulus (initial resistance to stretching) was 20.8 cN/dtex, the minimum value of the differential Young's modulus at an extension of 3-10% was 1.8 cN/dtex, and the elastic recovery following 10% elongation was 97.8%. The physical properties are shown in Table 1, and the stress-strain curve and the differential Young's modulus-strain curve are shown in Figure 3.

Moreover, when weaving was carried out as a 1/4 twill using this multifilament yarn as the warp/weft, the weaving characteristics and the woven material quality were good and the material possessed light stretchability.

### Example 2, Example 3

The same conditions were employed as in Example 1 except that the drawing rate was either 4350 m/min (draw ratio = 1.45) [Example 2] or 5000 m/min (draw ratio = 1.67) [Example 3]. The polyester yarn of Example 2 had a strength of 3.3 cN/dtex, which was lower than that of Example 1. Other characteristics were good in the same way as in Example 1. Moreover, while in the case of the polyester yarn of Example 3 the number of machine stoppages at the time of weaving increased to about twice when compared to Example 1, other properties were good.

### Example 4, Example 5

The same conditions were used as in Example 1 except that the relaxation factor between the second heated roller 5 and the cold roller 6 was adjusted to 6% [Example 4] or 18% [Example 5]. The polyester yarns of Example **4** and Example 5 were good in terms of their yarn production properties and woven material quality in the same way as in Example 1, and they had light soft stretchability. In particular, the woven material of Example 5 was even more outstanding in its softness than that of Example 1.

### Comparative Example 1

The same conditions were used as in Example 1 except that there was employed homo-PTT of intrinsic viscosity [η] 0.68. The spinnability of the polyester of Comparative Example 1 was poor and there were numerous yarn breakages in the drawing zone, so sampling was impossible.

### Comparative Example 2

The same conditions were used as in Example 1 except that the drawing rate was made 3900 m/min (draw ratio = 1.3). The polyester yarn of Comparative Example 2 had low strength and high extension, the strength being 2.9 cN/dtex and the extension 73.5%, and furthermore its elastic recovery following 10% stretching was low and the practical durability after forming a fabric was poor.

### Comparative Example 3, Comparative Example 4

The same conditions were used as in Example 1 except that the relaxation factor between the second heated roller **5** and the cold roller 6 was adjusted to 22% or 3%. In the case of the polyester yarn of Comparative Example 3 where the relaxation factor was 22%, there was considerable yarn oscillation over the second heated roller and, furthermore, yarn breakages occurred with yarn twisting around the second heated roller.

In the case of Comparative Example 4 where the relaxation factor was 3%, differences in properties arose between the package inner layer and outer layer due to occurrence of package tightening, and there were variations in thickness matching the package end face period. Furthermore, the weaving properties were poor and the quality of the dyed product was bad. Again, while the fabric possessed stretchability, it exhibited elongation characteristics where stretching was extremely difficult. The physical properties are shown in Table 1, and the stress-strain curve and the differential Young's modulus-strain curve are shown in Figure 4.

### Comparative Example 5

The same conditions were used as in Example 1 except that the drawing rate was made 5250 m/min (draw ratio = 1.75), cold roller 6 was removed and the relaxation factor was adjusted to 0%. In the case of Comparative Example 5, there was marked package tightening exceeding even that of Comparative Example 4 and, furthermore, the fabric obtained had stretch characteristics in which elongation was extremely difficult, and it was also inferior in its softness.

### Comparative Example 6

The same conditions were used as in Example 1 except that the first heated roller **4** velocity was adjusted to 1000 m/min and the second heated roller 5 velocity was adjusted to 3500 m/min (draw ratio = 3.5). Fabric comprising the polyester yarn of Example 6 showed good stretch characteristics in the same way as in Example 1, but dyeing unevenness arose in the dyed fabric which was thought to be due to yarn unevenness.

### Comparative Example 7

The same conditions were used as in Example 1 except that the second heated roller **5** was changed to a 0.8S (Rₘₐₓ: no more than 0.8µm) mirror surface roll. In Comparative Example 7, the travelling yarn in the relaxation zone between the second heated roller and cold roller **6** was unstable, and oscillation occurred on the second heated roller, with winding back on the roller and numerous yarn breakages occurring. Hence, compared to Example 1 the number of yarn breakages was about 10-fold.

### Example 6

The polyester yarn obtained in Example 1 was subjected to 2000 t/m (twist coefficient K: 14700) S/Z twisting to produce warp and weft yarns, and then a 1/4 twill fabric was produced. This was subjected to relaxation scouring at 98°C by the usual method, and then, intermediate setting carried out at 160°C. Subsequently, 15 wt% weight reduction was carried out with hot aqueous 3% NaOH solution, dyeing then performed and finish setting carried out. The fabric obtained was soft and its stretch properties were extremely outstanding.

In the table, 'relaxation factor' refers to the 'relaxation factor between the second heated roller and the cold roller 6'; the 'differential Young's modulus' refers to the 'minimum value of differential Young's modulus at an extension of **3** to 10%'; the 'elastic recovery' refers to the 'elastic recovery following 10% elongation'; the 'shrinkage stress' refers to the 'maximum value of shrinkage stress'; the 'peak temperature' refers to the 'temperature showing the maximum value of shrinkage stress'; the 'shrinkage CV%' refers to the 'CV% of the lengthwise direction continuous shrinkage'; and the 'woven fabric quality' refers to the 'quality of the appearance of the woven fabric after dyeing (functional evaluation)'.

### Industrial Applicability

With regard to the polyester yarn of the present invention and its method of production, as well as there being no package tightening in the yarn production stage and the package having a stable quality, it is possible to obtain woven fabric of low Young's modulus in the elastic recovery region and which is outstanding in its soft-stretch properties and softness.

**Table 1**

| | | Examples | | | | | Comparative Examples | | | | | | |
|---|---|---|---|---|---|---|---|---|---|---|---|---|---|
| | | 1 | 2 | 3 | 4 | 5 | 1 | 2 | 3 | 4 | 5 | 6 | 7 |
| Intrinsic viscosity | [η] | 0.96 | 0.96 | 0.96 | 0.96 | 0.96 | 0.68 | 0.96 | 0.68 | 0.96 | 0.96 | 0.96 | 0.96 |
| First HR velocity | m/min | 3000 | 3000 | 3000 | 3000 | 3000 | 3000 | 3000 | 3000 | 3000 | 3000 | 1000 | 3000 |
| Second HR velocity | m/min | 4800 | 4350 | 5000 | 4800 | 4800 | 4800 | 3900 | 4800 | 4800 | 5250 | 3500 | 4800 |
| Relaxation factor | % | 10.0 | 10.0 | 10.0 | 6.0 | 18.0 | 10.0 | 10.0 | 22.0 | 3.0 | 0.0 | 10.0 | 10.0 |
| Strength | cN/dtex | 3.6 | 3.3 | 3.7 | 3.7 | 3.4 | - | 2.9 | - | 3.5 | 3.8 | 3.7 | 3.6 |
| Extension | % | 50.5 | 59.2 | 43.2 | 42.0 | 57.8 | - | 73.5 | - | 44.3 | 26.5 | 45.4 | me |
| Young's modulus | cN/dtex | 20.8 | 19.4 | 21.5 | 21.7 | 19.8 | - | 18.9 | - | 21.5 | 28.6 | 21.0 | 20.8 |
| Differential Young's modulus | cN/dtex | 1.8 | 1.5 | 2.5 | 6.6 | 1.4 | - | 1.4 | - | 11.2 | 14.4 | 3.2 | 2.0 |
| Elastic recovery | % | 97.8 | 90.8 | 98.0 | 98.2 | 93.3 | - | 85.5 | - | 98,5 | 98.8 | 98.1 | 97.2 |
| Degree of crystallinity | % | 38 | 36 | 39 | 40 | 37 | - | 36 | - | 43 | 47 | 40 | 38 |
| Boiling water shrinkage | % | 6.7 | 6.2 | 7.5 | 8.0 | 6.5 | - | 5.8 | - | 8.7 | 10.0 | 7.3 | 6.6 |
| Shrinkage stress | cN/dtex | 0.17 | 0.13 | 0.19 | 0.20 | 0.15 | - | 0.11 | - | 0.25 | 0.33 | 0.19 | 0.17 |
| Peak temperature | °C | 168 | 169 | 170 | 170 | 167 | - | 167 | - | 171 | 171 | 172 | 167 |
| Shrinkage CV% | % | 2.8 | 3.7 | 3.0 | 3.8 | 3.2 | - | 4.2 | - | 7.6 | 7.9 | 5.2 | 4.5 |
| CF value | | 9.5 | 14.5 | 8.2 | 4.7 | 16.9 | - | 15.4 | - | 0.8 | 0.2 | 4.1 | 13.8 |
| Woven fabric quality | 4-stage evaluation | ⊚ | ○ | ⊚ | ○ | ⊚ | - | ○ | - | X | X | Δ | Δ |
| Stretch properties | 4-stage evaluation | ⊚ | ⊚ | ⊚ | ○ | ○ | - | Δ | - | X | X | ⊚ | ⊚ |

## Claims

1. Polyester yarn which is a multifilament yarn substantially comprising polytrimethylene terephthalate, and which has a strength from the stress-strain curve of at least 3 cN/dtex, a Young's modulus of no more than 25 cN/dtex, a minimum value of the differential Young's modulus at 3-10% extension of no more than 8 cN/dtex, an elastic recovery following 10% elongation of at least 90% and a CV value of the continuous shrinkage in the yarn lengthwise direction of no more than 4%.

2. Polyester yarn according to Claim 1 which has a Young's modulus of no more than 22 cN/dtex.

3. Polyester yarn according to Claim 1 or Claim 2, which has a minimum value of the differential Young's modulus at 3-10% extension of no more than 5 cN/dtex.

4. Polyester yarn according to any preceding Claim, which has a residual extension of at least 45%.

5. Polyester yarn according to any preceding Claim, which has an elastic recovery following 10% elongation of at least 95%.

6. Polyester yarn according to any preceding Claim, which has a degree of crystallinity of at least 30%.

7. Polyester yarn according to claim 6, which has a degree of crystallinity of at least 35%.

8. Polyester yarn according to any preceding Claim, which has a boiling water shrinkage of 3-15%, a maximum value of the shrinkage stress of no more than 0.3 cN/dtex and a temperature at which the maximum value of shrinkage stress is shown of at least 120°C.

9. Polyester yarn according to Claim 8, wherein the maximum value of the shrinkage stress is 0.15 to 0.25 cN/dtex.

10. Polyester yarn according to Claim 8 or Claim 9, wherein the temperature at which the maximum value of shrinkage stress is shown is at least 130°C.

11. Polyester yarn according to any preceding Claim, wherein the CF value is 1-30.

12. Polyester yarn according to Claim 11, wherein the CF value is 5-25.

13. Polyester yarn according to any preceding Claim, wherein the fineness of the individual filaments from which the polyester yarn is composed is no more than 3 dtex.

14. A woven fabric having a polyester yarn according to any preceding Claim as warp yarn and/or weft yarn in the form of a twisted yarn of twist coefficient 10,000 to 20,000.

15. A method of producing polyester yarn wherein multifilament yarn obtained by the melt spinning of polymer substantially comprising polytrimethylene terephthalate having an intrinsic viscosity [η] of at least 0.7 is hauled-off at a spinning rate of at least 2000 m/min and, without winding up, subjected to drawing and heat-treatment using a textured roll of surface roughness 1.5S-8S, after which it is continuously subjected to a relaxation heat treatment at a relaxation factor of 6 to 20% and wound up as a package.

16. A method according to Claim 15, which includes melt spinning of polytrimethylene terephthalate having an intrinsic viscosity [η] of at least 0.8.

17. A method according to Claim 15 or Claim 16, wherein the spinning is carried out at a temperature 20-50°C higher than the melting point of the polytrimethylene terephthalate.

18. A method according to any one of Claims 15 to 17, wherein the multifilament yarn is hauled-off at a spinning rate of at least 3,000 m/min.

19. A method according to any one of Claims 15 to 18, wherein the relaxation heat treatment is carried out at a relaxation factor of 8 to 18%.

20. A method according to any one of claims 15 to 19, wherein a textured roll of surface roughness 3.2S-6.3S is used in the drawing and heat-treatment.

21. A method according to any one of Claims 15 to 20, wherein the drawing temperature is 10-50°C higher than the glass transition temperature of polytrimethylene terephthalate.

22. A method according to any one of claims 15 to 21, wherein the drawing is conducted at a draw ratio for which the residual extension is at least 40%.

23. A method according to any one of Claims 15 to 22, wherein the heat setting and relaxation heat treatment are carried out at a temperature in the range 105-180°C.

## Patentansprüche

1. Polyestergarn, bei dem es sich um ein Multifilamentgarn handelt, das im Wesentlichen Polytrimethylenterephthalat umfasst und eine aus der Spannungs-Dehnungs-Kurve ermittelte Festigkeit von zumindest 3 cN/dtex, einen Elastizitätsmodul von nicht mehr als 25 cN/dtex, einen Mindestwert für den differenziellen Elastizitätsmodul bei 3-10 % Dehnung von nicht mehr als 8 cN/dtex, eine elastische Rückstellung nach 10 % Dehnung von zumindest 90 % und einen VarK-Wert der kontinuierlichen Schrumpfung in Garn-Längsrichtung von nicht mehr als 4 % aufweist.

2. Polyestergarn nach Anspruch 1, das einen Elastizitätsmodul von nicht mehr als 22 cN/dtex aufweist.

3. Polyestergarn nach Anspruch 1 oder Anspruch 2, das einen Mindestwert für den differenziellen Elastizitätsmodul bei 3-10 % Dehnung von nicht mehr als 5 cN/dtex aufweist.

4. Polyestergarn nach einem der vorangegangenen Ansprüche, das eine Restdehnung von zumindest 45 % aufweist.

5. Polyestergarn nach einem der vorangegangenen Ansprüche, das eine elastische Rückstellung nach 10 % Dehnung von zumindest 95 % aufweist.

6. Polyestergarn nach einem der vorangegangenen Ansprüche, das einen Kristallinitätsgrad von zumindest 30 % aufweist.

7. Polyestergarn nach Anspruch 6, das einen Kristallinitätsgrad von zumindest 35 % aufweist.

8. Polyestergarn nach einem der vorangegangenen Ansprüche, das eine Schrumpfung in siedendem Wasser von 3-15 %, einen Maximalwert für die Schrumpfspannung von nicht mehr als 0,3 cN/dtex und eine Temperatur, bei welcher der Maximalwert für die Schrumpfspannung auftritt, von zumindest 120 °C aufweist.

9. Polyestergarn nach Anspruch 8, worin der Maximalwert für die Schrumpfspannung 0,15 bis 0,25 cN/dtex beträgt.

10. Polyestergarn nach Anspruch 8 oder Anspruch 9, worin die Temperatur, bei welcher der Maximalwert für die Schrumpfspannung auftritt, zumindest 130 °C beträgt.

11. Polyestergarn nach einem der vorangegangenen Ansprüche, worin der KF-Wert 1-30 beträgt.

12. Polyestergarn nach Anspruch 11, worin der KF-Wert 5-25 beträgt.

13. Polyestergarn nach einem der vorangegangenen Ansprüche, worin die Feinheit der einzelnen Filamente, aus denen das Polyestergarn besteht, nicht mehr als 3 dtex beträgt.

14. Gewebe, das ein Polyestergarn nach einem der vorangegangenen Ansprüche als Kettfaden und/oder Schussfaden in Form eines verzwirnten Garns mit einem Verzwirnungskoeffizienten von 10.000 bis 20.000 aufweist.

15. Verfahren zur Herstellung eines Polyestergarns, worin ein Multifilamentgarn, das durch Schmelzspinnen eines Polymers erhalten wird, das im Wesentlichen Polytrimethylenterephthalat umfasst und eine Grenzviskosität [η] von zumindest 0,7 aufweist, mit einer Spinngeschwindigkeit von zumindest 2.000 m/min abgezogen wird und, ohne Aufwickeln, mittels einer strukturierten Walze mit einer Oberflächenrauigkeit von 1,5 S bis 8 S verstreckt und wärmebehandelt wird, wonach es kontinuierlich einer Relaxationswärmebehandlung mit einem Relaxationsfaktor von 6 bis 20 % unterzogen und zu einer Spule aufgewickelt wird.

16. Verfahren nach Anspruch 15, welches das Schmelzspinnen von Polytrimethylenterephthalat mit einer Grenzviskosität [η] von zumindest 0,8 umfasst.

17. Verfahren nach Anspruch 15 oder Anspruch 16, worin das Spinnen bei einer Temperatur von 20-50 °C über dem Schmelzpunkt des Polytrimethylenterephthalats durchgeführt wird.

18. Verfahren nach einem der Ansprüche 15 bis 17, worin das Multifilamentgarn mit einer Spinngeschwindigkeit von zumindest 3.000 m/min abgezogen wird.

19. Verfahren nach einem der Ansprüche 15 bis 18, worin die Relaxationswärmebehandlung bei einem Relaxationsfaktor von 8 bis 18 % durchgeführt wird.

20. Verfahren nach einem der Ansprüche 15 bis 19, worin eine strukturierte Walze mit einer Oberflächenrauigkeit von 3,2 S bis 6,3 S beim Verstrecken und bei der Wärmebehandlung eingesetzt wird.

21. Verfahren nach einem der Ansprüche 15 bis 20, worin die Verstreckungstemperatur 10-50 °C über der Glastemperatur von Polytrimethylenterephthalat liegt.

22. Verfahren nach einem der Ansprüche 15 bis 21, worin das Verstrecken bei einem Verstreckungsverhältnis durchgeführt wird, bei dem die Restdehnung zumindest 40 % beträgt.

23. Verfahren nach einem der Ansprüche 15 bis 22, worin die Thermofixierungs- und Relaxationswärmebehandlung bei einer Temperatur im Bereich von 105-180 °C durchgeführt wird.

## Revendications

1. Fil de polyester qui est un fil multifilamenteux comprenant sensiblement du polytriméthylène téréphtalate et qui a une résistance de la courbe effort-contrainte d'au moins 3 cN/dtex, un module de Young de pas plus de 25 cN/dtex, une valeur minimale du module de Young différentiel à 3-10% d'extension de pas plus de 8 cN/dtex, une récupération élastique à la suite de 10% d'allongement d'au moins 90% et une valeur CV du rétrécissement continu dans la direction longitudinale du fil de pas plus de 4%.

2. Fil de polyester selon la revendication 1, qui a un module de Young de pas plus de 22 cN/dtex.

3. Fil de polyester selon la revendication 1 ou la revendication 1 qui a une valeur minimale du module de Young différentiel à 3-10% d'extension de pas plus de 5 cN/dtex.

4. Fil de polyester selon toute revendication précédente qui a une extension résiduelle d'au moins 45%.

5. Fil de polyester selon toute revendication précédente qui a une récupération élastique à la suite d'un allongement de 10% d'au moins 95%.

6. Fil de polyester selon toute revendication précédente qui a un degré de cristallinité d'au moins 30%.

7. Fil de polyester selon la revendication 6 qui a un degré de cristallinité d'au moins 35%.

8. Fil de polyester selon toute revendication précédente qui a un rétrécissement dans l'eau bouillante de 3-15% et une valeur maximale de l'effort de rétrécissement de pas plus de 0,3 cN/dtex et une température à laquelle la valeur maximale de l'effort de rétrécissement est montrée d'au moins 120°C.

9. Fil de polyester selon la revendication 8 où la valeur maximale de l'effort de rétrécissement est de 0,15 à 0,25 cN/dtex.

10. Fil de polyester selon la revendication 8 ou la revendication 9 où la température à laquelle la valeur maximale de l'effort de rétrécissement est montrée est d'au moins 130°C.

11. Fil de polyester selon toute revendication précédente où la valeur de CF est de 1-30.

12. Fil de polyester selon la revendication 11 où la valeur de CF est de 5-25.

13. Fil de polyester selon toute revendication précédente où la finesse des filaments individuels dont le fil de polyester se compose n'est pas de plus de 3 dtex.

14. Etoffe tissée ayant un fil de polyester selon toute revendication précédente en tant que fil de chaîne et/ou fil de trame sous la forme d'un fil tordu d'un coefficient de torsion de 10000 à 20000.

15. Méthode de production d'un fil de polyester où un fil multifilamenteux obtenu par le filage en phase fondue d'un polymère comprenant sensiblement du polytriméthylène téréphtalate ayant une viscosité intrinsèque (η) d'au moins 0,7 est tracté à une vitesse de filage d'au moins 2000 m/min et, sans enroulement, est soumis à un étirage et un traitement thermique en utilisant un rouleau texturé d'une rugosité de surface de 1,5S-8S, et ensuite il est continuellement soumis à un traitement thermique de relaxation à une facteur de relaxation de 6 à 20% et est enroulé en un ensemble.

16. Méthode selon la revendication 15 qui comprend le filage en phase fondue de polytriméthylène téréphtalate ayant une viscosité intrinsèque (η) d'au moins 0,8.

17. Méthode selon la revendication 15 ou la revendication 16 où le filage est effectué à une température de 20-50°C plus élevé que le point de fusion du polyméthylène téréphtalate.

18. Méthode selon l'une quelconque des revendications 15 à 17 où le fil multifilamenteux est traité à une vitesse de filage d'au moins 3000 m/min.

19. Méthode selon l'une quelconque des revendications 15 à 18 où le traitement thermique de relaxation est effectué à un facteur de relaxation de 8 à 18%.

20. Méthode selon l'une quelconque des revendications 15 à 19 où un rouleau texturé d'une rugosité de surface de 3,2S-6,3S est utilisé dans l'étirage et le traitement thermique.

21. Méthode selon l'une quelconque des revendications 15 à 20 où la température d'étirage est de 10-50°C plus élevée que la température de transition vitreuse du polytriméthylène téréphtalate.

22. Méthode selon l'une quelconque des revendications 15 à 21 où l'étirage est entrepris à un rapport d'étirage pour lequel l'extension résiduelle est d'au moins 40%.

23. Méthode selon l'une quelconque des revendications 15 à 22 où la prise à chaud et le traitement thermique de relaxation sont effectués à une température comprise entre 105-180°C.
